

## UNITED STATES PATENT OFFICE

2,190,848

## DYEINGS

Siegfried Petersen, Otto Bayer, and Carl Taube,  
Leverkusen-I. G. Werk, Germany, assignors to  
General Aniline & Film Corporation, a cor-  
poration of Delaware

No Drawing. Application May 20, 1937, Serial  
No. 143,726. In Germany May 30, 1936

9 Claims. (CL 8—75)

The present invention relates to a process of improving dyeings on textile fibers and similar material.

It is known that in many cases dyeings of organic dyestuffs, especially such as contain free carboxylic or sulfonic acid groups, can be improved by causing the said dyestuffs to interact on the dyed material with organic bases like amines, quaternary ammonium compounds or soluble salts thereof. By such processes the dyestuffs are more solidly fixed on the dyed material so that the dyeings will be of better fastness to water, to washing and the like. The said treatment has been carried out either by 15 aftertreating the dyed material or by pretreating the material and thereafter dyeing it with direct or acid dyestuffs.

We have now found that still better results are obtained by employing for the said purpose such organic bases as have combined therewith a metal in complex form but as are still capable of forming salts with acids. By our new process, for instance, in many cases the fastness of the dyeings to water will be materially increased 25 whilst in these and other cases the treated dyeings will be much faster to the action of light. Moreover, often a remarkable change in color of the treated dyeing has been observed thus yielding for instance a deeper shade or a more 30 valuable tint of increased fastness. The process of our invention has proved to be especially suitable for improving dyeings of substantive dyestuffs on cellulosic textile fibers like cotton or artificial silk from regenerated cellulose. 35 These and other objects and results of our invention will be more fully illustrated by the following description thereof.

The metal complex compounds to be used according to our invention are derived from organic bases which may belong to the aliphatic or cyclic series. As examples we may mention the metal complex compounds of guanidino, of thiourea, of o-phenanthroline, of phenylene diamines, of 2,2'-dipyridyl, of 8-amino-quinoline, of 8-amino-quinaldine and the like. The metals suitable for preparing the compounds to be used according to our invention are of the type which easily forms complex compounds with organic bases, for instance, chromium, iron and especially copper.

The process of our invention may be carried out by aftertreating the dyed fibers with an aqueous solution of one of the said complex metal compounds; if desired, the solution may be weakly acid or alkaline. In another modifica-

tion of our process forming of the metal complex compound and aftertreating of the dyeing is performed in one and the same bath. Our invention will be apparent in more detail from the following examples without, however, being limited thereto:

*Example 1*

The aqueous solution of the copper complex of the compound of the following constitution:



is used for the aftertreatment of a 2% dyeing with Diamine Pure Blue FF (comp. Col. Ind. No. 517). On aftertreating for half an hour, which aftertreatment can also be effected in an acetic acid or an alkaline solution, there is obtained in contrast to the non-aftertreated solution an essentially greener shade. The after-treated dyeing is distinguished by its fastness to washing and light.

A similarly improved fastness to water and washing is obtained on aftertreating in the usual manner dyeings with Congo Red (Co. Ind. No. 370) or with Direct Deep Black EW.

The above mentioned compound is obtainable by reacting upon 1 mol of cyanuric chloride with 1 mol of m-amino-phenyl-trimethyl-ammoniumchloride and 1 mol of 5-amino-8-hydroxy-quinoline.

*Example 2*

A 2% dyeing on cotton with the dyestuff which is obtained by coupling in an alkaline medium diazobenzene and diazotized 2-naphthylamine-6-sulfonic acid with the urea of I-acid, is treated, after washing, for half an hour at 30° C. with an aqueous solution of the complex compound prepared from cupric sulfate and 8-amino-quinaldine (obtainable by stirring an alcoholic solution of 8-amino-quinaldine into an aqueous cupric sulfate solution). By this treatment the scarlet red dyeing becomes dark brown and acquires a good fastness to washing.

On treating dyeings of Diamine Green B (comp. Col. Ind. 1st edition, No. 593) in the manner described in the preceding paragraph, these dyeings become essentially faster to washing and deeper.

*Example 3*

A 2% dyeing of Diamine Pure Blue FF is

5

10

20

25

30

35

40

45

50

55

treated for half an hour in a bath which contains dissolved the copper complex obtainable from cupric sulfate and 8-amino-quinoline. Thereby the dyeing becomes somewhat more 5 dull and faster to washing.

*Example 4*

10 Cotton which has been dyed with 7% of Sirius Black L (comp. Schultz, Farbstofftabellen, Er- gänzungsband, 1934, page 132) is treated in an aqueous solution at 30° C. prepared from o-phenanthroline-cupric-chloride (obtainable from o-phenanthroline

15



and cupric chloride). The dyeing becomes more 20 greenish and is improved as regards its fastness to washing.

Instead of the copper complex compound of o-phenanthroline there can be used the copper complex compound of nitro-o-phenanthroline, which is obtainable by nitration, or of the reduction product thereof, or of the compound obtainable by causing 1 mol of 2,3-diamino-naphthalene, and 2 mols of glycerine to react according to the method of Skraup.

30

*Example 5*

The fastness to water and washing of cotton dyeings prepared with Diamine Green B are improved on aftertreating the same with solutions of the complex salts prepared from cupric chloride 35 with 1 or 2 mols of  $\alpha,\alpha'$ -dipyridyl.

The fastness to washing of the dyeings is also improved by using the corresponding complex iron salts.

*Example 6*

40 Cotton dyed with Direct Deep Black EW extra is aftertreated with the solution of the cupric complex salt of NN'-tetramethyl-o-phenylene-diamine. Such solutions may, for instance, be obtained by adding 1 mol of base and 1 mol of copper acetate in alcohol and dilution with water of this alcoholic solution which, if desired, may have been filtered. The fastness to water of the aftertreated dyeings is improved.

50 A similar effect is obtained, for instance, by the copper complex solution of N-monomethyl-o-phenylenediamine.

We claim:

1. In the process of improving dyeings of organic dyestuffs containing free acid groups on textile fibers the modification which comprises causing the dyed fibers to interact with a complex metal compound of a cyclic base containing at least two basic nitrogen atoms which metal compound is capable of forming salts with acids.

2. In the process of improving dyeings of organic dyestuffs containing free acid groups on textile fibers the modification which comprises causing the dyed fibers to interact with a complex copper compound of a cyclic base containing at least two basic nitrogen atoms which copper compound is capable of forming salts with acids. 5

3. In the process of improving dyeings of organic dyestuffs containing free acid groups on cellulosic fibers the modification which comprises 10 causing the dyed fibers to interact with a complex copper compound of a cyclic base containing at least two basic nitrogen atoms which copper compound is capable of forming salts with acids.

4. In the process of improving dyeings of organic dyestuffs containing free acid groups on cellulosic fibers the modification which comprises causing the dyed fibers to interact with a complex copper compound of a cyclic organic base 20 containing at least two basic nitrogen atoms which copper compound is capable of forming salts with acids.

5. In the process of improving dyeings of organic dyestuffs containing free acid groups on cellulosic textile fibers the modification which comprises treating the dyed fibers with an aqueous solution of a complex copper compound of a N-heterocyclic base containing at least two basic nitrogen atoms which copper compound is capable of forming salts with acids. 30

6. In the process of improving dyeings of organic dyestuffs containing free acid groups on cellulosic fibers the modification which comprises treating the dyed fibers with an aqueous solution 35 of a complex copper compound of 8-amino-quinoline which copper compound is capable of forming salts with acids.

7. In the process of improving dyeings of organic dyestuffs containing free acid groups on cellulosic textile fibers the modification which comprises treating the dyed fibers with an aqueous solution 40 of a complex copper compound of 8-amino-quinoline which copper compound is capable of forming salts with acids.

8. Textile fibers dyed with organic dyestuffs containing free acid groups, said dyed fibers being combined with a complex metal compound of a cyclic base containing at least two basic nitrogen atoms which metal compound is capable of 50 forming salts with acids.

9. Cellulosic textile fibers dyed with organic dyestuffs containing free acid groups, said dyed fibers being combined with a complex copper compound of a N-heterocyclic base which copper compound is capable of forming salts with acids. 55

SIEGFRIED PETERSEN.

OTTO BAYER.

CARL TAUBE.

60